# EUROPEAN PATENT SPECIFICATION

(11) **EP 2 729 286 B1**
(45) Date of publication and mention of the grant of the patent: **18.12.2019**
(21) Application number: 12807966.2
(22) Date of filing: 03.07.2012
(51) Int. Cl.: B05C 11/02, B28B 19/00, B05C 9/12

(54) **VIBRATING FINISHING PLATE TECHNOLOGY**
VIBRATIONSPLATTE FÜR ENDBEARBEITUNGSVERFAHREN
TECHNOLOGIE DE FINITION PAR PLAQUE VIBRANTE

(30) Priority: 04.07.2011 US 201161504279 P
(43) Date of publication of application: 14.05.2014
(73) Proprietor: ShawCor Ltd., Toronto, Ontario M9W 1M7 (CA)
(72) Inventor: REIZER, Kevin, Ascot Berkshire SL5 0PS (GB); ABUSLAND, Vidar, Conroe, Texas 77301 (US); ZACARIAS, Philip De Sousa, Mississauga, Ontario L5R 2T2 (CA); FRAME, Adam Donaldson, Prestonpans East Lothian Lothian EH32 9NW (GB)
(74) Representative: Mewburn Ellis LLP
(86) International application number: PCT/CA2012/050452
(87) International publication number: WO 2013/003956

(56) References cited:
- CA-A1- 1 216 505
- CN-Y- 201 189 699
- DE-A1- 2 214 155
- DE-B- 1 120 966
- FR-A1- 2 315 374
- FR-A1- 2 427 187
- FR-A1- 2 540 779
- JP-A- H08 300 340
- SU-A1- 494 558
- US-A1- 2007 026 172

## Description

### FIELD

The invention relates to a device and a method for vibrationally finishing an impinged concrete coating on a pipe.

### BACKGROUND

Typically, an impingement process is used for offshore concrete coating of a pipe. The process involves batched material passing through two large rubberized rollers at high speed to build up the required concrete thickness on the pipe. The impingement process creates a surface which is uneven (non-uniform), rough and undulating due to a number of reasons, including layer overlap, variations in the mass of the feed delivered to the rollers, rebound and surface fall-off.

The non-uniform surface of the concrete appears porous, along with a reduced average density of the concrete in the outer layers of the coating. Decreasing the variation in surface profile can allow for a reduction in concrete thickness or the application of concrete which has a higher density - either the mass of concrete or the amount of iron ore in the concrete can be decreased to obtain the desired negative buoyancies.

Also, when phi tapes measuring systems are used to measure the diameter of such non-uniform pipes, the measurements are essentially peak-to-peak and therefore the diameter is greater than the actual diameter. Decreasing the variation in the profile of the surface can provide more accurate determination of pipe diameter and therefore better buoyancy estimates.

In addition to the above, the non-uniform surface formed from an impinged concrete coated pipe leads to dust generation during the process of laying the pipe. The impinged concrete surfaces shed a significant amount of fine concrete material because the outer layers are friable. According to a marketing survey, it costs lay barge operators about $2 million annually to remove detritus generated by impinged concrete. Concrete which has a smoother and denser surface will generate less detritus and reduce disposal costs for lay barge operators.

The smoothening of pipes can have a tertiary benefit which is the reduction of the coefficient of friction between the pipe and the seabed. In some instances, problems have been reported when the friction between the pipes and the seabed can lead to significant dust generation.

CN 201189699Y describes an apparatus for smoothing a concrete pipe comprising a scraper mounted on an arm, with the arm mounted on a frame. Also described are methods for smoothing a concrete pipe, and a pipe obtained from such a method.

FR 2315374 describes an apparatus for smoothing the coating on a prestressed concrete pipe comprising a vibrating plate mounted on an arm. The vibrating plate acts in the plane which is tangential to the finished concrete surface. Also described are methods for smoothing the coating on a prestressed concreate pipe, and a pipe obtained from such a method.

Hence, there is a need in the art for a process for finishing the concrete coating surface on a pipe to obtain a smoothened coating. The finishing of an impinged concrete coating can address a number of concerns, as noted above. In addition, there is a need in the art for a device for carrying out the process to finish and provide a smoothened concrete coated pipe.

### SUMMARY OF THE INVENTION

In one aspect, the invention relates to a pipe coating finishing device comprising:
- one or more frames having a first arm and a second arm;
- a scraper coupled to a first arm for engaging a pipe to remove material in excess of a maximum pipe diameter; and
- a vibrating plate coupled to a second arm for compacting an impinged concrete coating on the pipe,
wherein the vibrating plate comprises raised edges for preventing the vibrating plate edges from digging into the impinged concrete coating.

In another aspect the invention relates to a process for finishing an impinged concrete coating on a pipe with a device according to the invention, the process comprising the steps of:
- scrapping material in excess of a maximum coated pipe diameter; and
- vibrationally compacting a surface of the impinged concrete coated pipe to form a smoothened concrete coated pipe.

### BRIEF DESCRIPTION OF THE DRAWINGS

Reference will now be made, by way of example, to the accompanying drawings which show example embodiments of the present application, and in which:
Figure 1 shows a front elevational schematic view of an embodiment of the device according to the invention;
Figure 2 shows a perspective schematic view from the vibrating plate side of an embodiment of the device according to the invention;
Figure 3 shows a perspective view from the scraper side of an embodiment of the device according to the invention;
Figure 4 shows a top view of an embodiment of the device according to the invention;
Figure 5 shows a side elevational view of an embodiment of the device according to the invention;
Figure 6 shows a perspective view of a set-up of a vibrational finishing plate device according to another embodiment of the invention;
Figure 7 shows a picture of a impinged concrete coated pipe undergoing a vibrationally finishing plate process according to the invention;
Figure 8 shows an electric vibrator having eccentric weights used in an embodiment according to the invention;
Figure 9 shows a close-up picture of a pipe showing the surface of an impinged concrete coated pipe along with a vibrationally finished concrete coated pipe after undergoing the process according to an embodiment of the invention;
Figure 10 shows another close-up picture of a pipe showing the surface of an impinged concrete coated pipe along with a vibrationally finished concrete coated pipe after undergoing the process according to an embodiment of the invention;
Figure 11 shows a picture of a surface of a vibrationally finishing concrete coated pipe after undergoing through the process according to the invention;
Figure 12 shows the iron ore sieve analysis used in coating the pipe in accordance with the process of the invention;
Figure 13 discloses the profile of test pipes after finishing with a vibrating finishing plate (VFP) device used in accordance with the process of the invention;
Figure 14 discloses the outer diameter (OD) profile of pipe M1 before and after undergoing the process according to the invention;
Figure 15 discloses the outer diameter (OD) profile of pipe G1 before and after undergoing the process according to the invention;
Figure 16 discloses the densities and thickness of various pipes having an impinged concrete coating;
Figure 17 a front elevational schematic view of another embodiment of the device according to the invention;
Figure 18 a top elevational schematic view of another embodiment of the device according to the invention;
Figure 19 a front elevational schematic view of a further embodiment of the device according to the invention;
Figure 20 a front elevational schematic view of another further embodiment of the device according to the invention;

Similar reference numerals may have been used in different figures to denote similar components.

### DESCRIPTION

As discussed above, the invention relates to a pipe coating finishing device (1) and a process for finishing an impinged concrete coating (32) on a pipe (12) with the pipe coating finishing device (1).

Figures 1-7 show a pipe coating finishing device (1) that contains a frame (2) having a first arm (4) and a second arm (6). Coupled to the first arm (4) at the pipe end of the first arm (10) is a scraper (8), which is used to remove any impinged concrete coating material that exceeds a pre-set maximum concrete coated pipe diameter. While the second arm (6) is coupled to a vibrating plate (14) at the pipe end of the second arm (16), for compacting an impinged concrete coating on the pipe (32). As shown in figures 1-5, both the first arm (4) and the second arm (6) are coupled to a single frame (2) structure. However, separate frame structures can be used (as shown in figures 16-20), where a first arm (4) is coupled to a first frame structure (not shown) and the second arm (6) is coupled to a second frame (2) structure (shown in figures 16-20). As described herein, such embodiments are intended to be covered by the frame (2) and the first arm (4) and the second arm (6), disclosed herein.

The vibrating plate (14) used in the device (1) is able to vibrate at sufficiently high frequency and apply sufficient pressure to compact the impinged concrete coating on the pipe (32). In one embodiment of the invention, the vibrating plate (14), as disclosed in the embodiment shown in the figures, has a convex surface that faces away from the pipe and a concave surface (22) that faces the impinged concrete coated pipe (32). In a further embodiment of the invention, the concave surface (22) of the vibrating plate (14) has a radius of curvature to allow nearly the entire concave surface (22) to contact the outer surface of the impinged concrete coated pipe (32). Such a concave structure can assist in uniformly compacting and finishing the impinged concrete coating on the pipe.

In one embodiment of the invention, the vibrating plate (14) is provided with a vibrator (18) (Figures 1, 2, 8 and 16-20), which permits the vibrating plate (14) to vibrate at a desired frequency. In a further embodiment according to the invention, the vibrating plate (14) vibrates at a frequency from about 1500 to about 18000 vpm. In another embodiment according to the invention, the vibrating plate vibrates at a frequency from about 3500 to about 12000 vpm. In a still further embodiment, the vibrating plate (14) vibrates at a frequency from about 6500 to about 9000 vpm. In another embodiment, the vibrating plate (14) vibrates at a frequency of about 3000 vpm.

In an embodiment according to the invention, the vibrating plate (14) applies a static pressure on the impinged concrete coated pipe (32) to compact and provide finishing to the concrete coating. In one embodiment, pressure can be applied by using weights (34) on the vibrating plate (14) (figures 19 and 20). In another embodiment, pressure can be used by connecting the vibrating plate (14) to a hydraulic system (figures 16-18). The amount of pressure applied can also vary depending upon the properties of the coated concrete and the vibrating plate (14). In one embodiment, the amount of static thrust force applied ranged from about 20.68 to about 1379 kPa (about 3 to about 200 psi). In another embodiment, the amount of static thrust force applied ranged from about 517.1 to about 1034 kPa (about 75 to about 150 psi), and values in between. In a still further embodiment, the amount of down force applied using about 300 to 600 kPa (3 to 6 bar) of pressure ranged from about 4 to 12 kN.

As the vibrating plate (14) vibrates, the impinged concrete coating is compacted to obtain a smoothened surface. The size of the vibrating plate can vary depending upon pipe and the desired process. In one embodiment, for example and without limitation, the width of the vibrating plate (14) is such that any given area of the impinged concrete coating is compacted and finished at least twice by the vibrating plate (14). Other embodiments, where compacting and finishing on any given area is performed multiple times, such as, for example and without limitation, three, four, five or more, by the vibrating plate are also encompassed by the present invention. The number of times, compacting and finishing on any given area on the concrete coated pipe is performed can depend on the pipe dimensions, pipe line speed, pipe rotation. In one embodiment, for example, where the pipe has an outer diameter (OD) of 914.4mm and 23 mm wall thickness, and where the concrete coating thickness was 75 mm, the linear speed of the pipe was 7.5 m/min and rotation was 20.69 rpm. Based on this, it was determined that the coating surface rotates at 1.49 revolutions under the area of the finishing plate.

During the compacting and finishing process, to avoid the edges of the vibrating plate from digging into the compacted and finished concrete coating, the edges of the vibrator plates are raised (20) (see Fig. 1 and 16-20). This provides a vibrator plate (14) with smoothened edges and also assists in producing a smoothened concrete coated pipe.

The scraper (8) and the vibrating plate (14) are positioned on the pipe (12) to allow the scraper (8) to first contact the impinged concrete coating (32) on the pipe (12), so as to remove concrete that is in excess of a maximum concrete coated diameter. Subsequently, after an area of the impinged concrete coating (32) on the pipe (12) undergoes scrapping, it then contacts the vibrating plate (14) for smoothening and finishing the concrete coating on the pipe. The leading scraper takes the larger surface undulations and particles out, and the VFP which follows is able to smooth this pre-conditioned surface.

The positioning of the scraper (8) and the vibrating plate (14) on the impinged concrete coated pipe (32) can be such that both the scraper (8) and the vibrating plate (14) are positioned in-line along the length of the pipe (12). One possible way to achieve this, is to have the scrapper and the vibrating plates on separate frames, such as embodied in Figures 16-20. However, the impinged concrete coating and finishing process can also be carried out concurrently, so as to allow impingement of the pipe prior to scrapping and finishing the concrete coated pipe. In such a process, the pipe is rotated and moved along the length of the pipe while being impinged by a concrete coating. In such an embodiment, the vibrating plate (14) and the scraper (8) are positioned in-line along an axis perpendicular to the longitudinal axis of the pipe (12). Therefore, as the pipe (12) is impinged with a concrete coating, rotated and moved along the length of the pipe (12), it is also scrapped and finished to obtain a smoothened concrete coating on the pipe (12) (Figures 1-6).

In addition to the above and as shown in the figures, the scraper (8) and the vibrating plate (14) can be positioned on the pipe (12) to be adjacent to each other, as shown in Figures 1-7. In one embodiment, the scraper (8) is positioned below and the vibrating plate (14) is positioned above a plane diametrically dissecting the pipe (12). The plane that diametrically dissects the pipe (12) can lie normal to the ground surface. In a further embodiment, the scraper (8) and the vibrating plate (12) are symmetrically positioned about the plane diametrically dissecting the pipe (12). In the embodiments disclosed in the figures, the scraper (8) and vibrating plate (14) are positioned at an angle of about 30° measured from the pipe centre. However, other angles, such as about 20°, 25°, 35° or 40° may also be considered acceptable. While in the embodiments disclosed in Figures 16-20, the vibrating plate (14) and/or the scrapper (not shown) can lie in the plane that diametrically dissects the pipe (12), with the plane being normal to the ground surface.

The step of impinging a concrete coating on the pipe (12) is not particularly limited. In one embodiment, for example and without limitation, impingement of the concrete coating on the pipe (12) is carried out by use of impingement rollers. In the embodiment disclosed above, where coating, scrapping and finishing is carried out concurrently, the impingement rollers can be positioned adjacent to the vibrating plate and/or the scraper.

The scraper (8) used in accordance with the invention should be able to remove excess impinged concrete coating on the pipe (12) without damaging the concrete coating. In one embodiment, for example, the scraper (8) is provided with a first end plate (24), a second end plate (26) and a plurality of rods (28) connecting the first end plate (24) to the second end plate (26). The plurality of rods (28) extending from the first end plate (24) to the second end plate (26) can be positioned to extend along the length of the pipe (12), to allow scrapping the excess impinged concrete coating on the pipe (12), as the pipe (12) rotates and moves along the length of the pipe (12). Moreover, the plurality of rods (28) can be so arranged that they together define a curved plane having a radius of curvature equal to the set maximum radius of the coated pipe (12).

The above-noted concurrent steps of impinging the concrete coating, scrapping the excess concrete coating and finishing the concrete coating, the process can be carried out a surface speed of the pipe (12) sufficient to adequately smoothen and finish the pipe (12). In one embodiment, the surface speed of the pipe is from about 50 to about 100 meters/min, and values in between, such as, about 60, about 70, about 75 and about 80 meters/min.

In a further embodiment in accordance with the specification, water can be applied during the process for finishing an impinged concrete coating on a pipe. The application of water can help with the scrapping step, the vibrationally finishing step, or both. The rate of water application in the process can vary. In one embodiment, for example, the rate of water application ranged from about 0.030 to 1.000 L/m². In another embodiment, the rate of water application ranged from, for example, about 0.047 to 0.071 L/m².

Using the device and method disclosed herein, concrete coated pipes having a smoothened profile were obtained. To evaluate the smoothness of the coating on the pipe, the average depth of indentation on the concrete coated pipes were measured. In one embodiment, for example, the average depth of the indentation measured on the coating was below 5 mm. In another embodiment, the average depth of the indentation measured on the coating ranged from, for example, about 2.5 to 4.96 mm. In a further embodiment, the average depth of the indentation measured on the coating ranged from about 3% to about 6.5%.

The device and process according to the invention leads to a concrete coated pipe having a smoothened finished surface, as shown in figures 7 and 9-11. In addition, the amount of detritus generated can be significantly lowered, which can address some of the health and safety hazards associated with the impinged concrete coated pipes in present use. In one embodiment, for example, the pipes obtained using the process disclosed herein, generated about 200, 300, 400, 500%, 600% or 700%, and values in between, less detritus than that generated using an impinged concrete coated pipe.

### DESCRIPTION OF EXAMPLE EMBODIMENTS

The application will be described by way of a non-limiting example to disclose the process of obtaining a smoothened and finished concrete-coated pipe.

### Materials and Methods

The pipes were 111.76 cm (44 inches) in diameter and had a wall thickness of 23.3 mm. The anticorrosion coating was 6 mm (modified) asphalt. Plastic spacers (65 mm) positioned the 8 mm rebar cage in the middle third of the 110 mm concrete coating. Eight strands of fibrillated polypropylene twine were wrapped around the pipe to restrain the concrete and prevent disbondment or fall-off. The twine stands are typically positioned within the first 10 mm of the concrete surface and approximately 5 kg of tension was applied on each strand of twine.

A concrete mixture with a target density of 3400 kg/m³ and containing 550 kg/m³ Portland cement was used. The range of moisture content acceptable for coating was 4.5 to 5.1%. The Portland cement was supplied by Norcem AS Norway, the magnetite from Minelco AB Sweden. The sieve analysis data for the aggregate is shown in Figure 12.

For the diameter of pipe and concrete thickness used in this test program, the coating time and surface speed selected were 165 seconds and 72 meters/minute, respectively.

The vibrating finishing plate used in this test program was 540 mm wide x 500 mm long. The width of the plate was based on the design criteria that any given area of the concrete surface would be compacted and finished twice by the vibrating finishing plate (VFP). Two Dynapac ER 305 electric vibrators were used (Figure 8). Alternately, other vibrators such as VIBCO US-450T-230V can also be used. The vibrators were mounted parallel to each other on the plate at opposite ends of the plate (Figure 6). The rotors in the vibrators operated at a fixed speed of 3000 rpm and the internal weights (Figure 8) were set for the maximum force of 3000 Newtons. The vibrators were electrically connected such that the rotors inside the vibrator were counter rotating with respect to each other - one shaft rotated clockwise and the other anti-clockwise - this produced a reciprocating motion that was predominantly normal to the surface of the concrete. A 100 mm diameter pneumatic cylinder was used to apply a static pressure to the plate. For the tests in this program the maximum pressure of 699.82 kPa (101.5 psi) was used. The estimated static thrust force on the plate was 20.68 kPa (3 psi). The vibrating finishing plate was mounted just in front of the impingement rollers and in line with the scraper. The scraper and VFP contacted the pipe at approximately 28° before and after top-dead-center, respectively (Figures 6 an 7).

The VFP was evaluated by first coating the pipe without the VFP and measuring the outside diameter of the pipe via the optical OD measuring system. After the pipe was coated, manual measurements were immediately taken and recorded. The pipe was repositioned and passed through the HeviCote system again with a normal production surface speed of 72 meters/min. but with the VFP on the pipe running with maximum pressure and amplitude. Again, OD measurements were taken by the optical system and manually.

Profile analysis was performed on the smoothed surface after hardening by measuring the depth of the surface relative to a 1.95 meter long aluminum straight edge (Figure 13) every 10 cm. The straight edge was moved along the length of the pipe until the full length was profiled.

### Results

Figures 14 and 15 show the OD profiles before and after the VFP. According to manual measurements, the OD was reduced 3.2 and 1.4 mm for pipes M1 and G1, respectively. For measurements by the optical system, the OD was reduced by 1.9 and 1.3 mm.

The profile of the surface for both pipes after finishing and curing is given in Figure 13. Due to the weak nature of uncured concrete and the loss of surface moisture it was not possible to determine a profile of the freshly impinged pipe before exposure to the VFP. As reference and for comparison, the profile for various pipes manufactured is given in Figure 16. The average variation in depth of unfinished impinged concrete according to profile measurements is generally 4-5 mm and for finished pipes about 3.4 mm (∼ 1 mm reduction).

Theoretical analysis using the profile data for unfinished and finished pipes indicates that this variation reduces the overall density of the concrete on the pipe and requires that concrete with a higher density be applied. Figure 11 illustrates the effect of finishing on the density of the (applied) concrete required to meet the target density on the pipe. Assuming a 50 mm concrete coating thickness and a target density of 3044 kg/m³, the density of the applied concrete for unfinished pipes must be at least 3300 kg/m³, and for finished pipe the density needs to be a minimum of 3167 kg/m³. Approximately 9% less iron ore (4800 kg/m³ density) is needed per metric ton of concrete when the density is decreased from 3300 to 3167 kg/m³.

A trial to mimic the handling a pipe will experience on a typical laybarge firing line was performed. This was done by repeatedly running the test pipes over a fixed set of rollers for a total of 20 passes. One pass is considered a movement of 1m in the forward direction. The dust generated was collected by two sources, after the 20 passes. The smaller dust particles were sucked up via a large industrial vacuum whilst the heavier particles which were not captured by the vacuum fell onto a collection plate. The two dust collection sources were weighted and analyzed separately. Four tests were conducted on each pipe at the 12, 3, 6 and 9 o'clock positions on the pipe, VFP and impinged pipe, gathering a total of 80 passes, 20 passes per individual test. Two pipes were used, one impinged pipe which acted as the "control pipe", and one VFP pipe. The control pipe provided a baseline to compare the dust levels generated by the VFP pipe. Dust levels utilizing the VFP decreased 471% compared to the impinged concrete pipe. This is a significant reduction in dust compared to normal impinged concrete and occurred in all gradation spectrums.

The trials conducted demonstrated that the VFP can significantly improve the uniformity of the surface and thereby reduce the thickness of the concrete coating, without loss of material.

Certain adaptations and modifications of the described embodiments can be made. Therefore, the above discussed embodiments are considered to be illustrative and not restrictive.

## Claims

1. A pipe coating finishing device (1) comprising:
- one or more frames (2) having a first arm (4) and a second arm (6);
- a scraper (8) coupled to a first arm 4) for engaging a pipe (12) to remove material in excess of a maximum pipe diameter; and
- a vibrating plate (14) coupled to a second arm (6) for compacting an impinged concrete coating (32) on the pipe (12),
wherein the vibrating plate (14) comprises raised edges (20) for preventing the vibrating plate (14) edges from digging into the impinged concrete coating.

2. The pipe coating finishing device (1) according to claim 1, further comprising a vibrator (18) coupled to the vibrating plate (14).

3. The pipe coating finishing device (1) according to claim 1 or 2, wherein the vibrating plate (14) has a concave surface (22) having a radius of curvature to allow the entire concave surface (22) of the vibrating plate (14) to contact an outer surface of the impinged concrete coated pipe (12).

4. The pipe coating finishing device (1) according to any one of claims 1 to 3, wherein the vibrating plate (14) and the scraper (8) are positioned in-line along an axis perpendicular to the longitudinal axis of the pipe (12).

5. The pipe coating finishing device (1) according to any one of claims 1 to 4, wherein the scraper (8) has a first end plate (24), a second end plate (26), and a plurality of rods (28) connecting the first end plate (24) to the second end plate (26); and the plurality of rods (24) defining a curved plane having a radius of curvature equal to a set maximum radius of the coated pipe (12).

6. The pipe coating finishing device (1) according to any one of claims 1 to 5, further comprising impingement rollers positioned adjacent to the vibrating plate (14) and scraper (8).

7. The pipe coating finishing device (1) according to any one of claims 1 to 6, wherein the scraper (8) is positioned below and the vibrating plate (14) is positioned above a plane diametrically dissecting the pipe (12).

8. The pipe coating finishing device (1) according to claim 7, wherein the scraper (8) and vibrating plate (14) are symmetrically positioned about the plane diametrically dissecting the pipe (12).

9. The pipe coating finishing device (1) according to claim 7 or 8, wherein the scraper (8) and vibrating plate (14) are positioned at an angle of about 30° measured from the pipe (12) centre.

10. A process for finishing an impinged concrete coating on a pipe (12) with a device (1) as defined in any one of claims 1 to 9, the process comprising the steps of:
- scrapping material in excess of a maximum coated pipe diameter; and
- vibrationally compacting a surface of the impinged concrete coated pipe (32) to form a smoothened concrete coated pipe (12).

11. The process for finishing an impinged concrete coating on a pipe according to claim 10, further comprising the step of:
- impinging a concrete coating on a surface of a pipe, prior to the scrapping and vibrationally compacting steps, to obtain the impinged concrete coated pipe (32).

12. The process for finishing an impinged concrete coating on a pipe according to claim 10 or 11, wherein the vibrating plate (14) applies a pressure of from about 34.47 to about 5516 kPa (about 5 to about 800 psi), wherein the vibrating plate preferably vibrates at a frequency from about 1500 to about 18000 vpm.

13. The process for finishing an impinged concrete coating on a pipe according to any one of claims 10 to 12, wherein the vibrating plate (14) has a width to allow compacting, at least twice, a surface of the impinged concrete coated pipe (32).

14. The process for finishing an impinged concrete coating on a pipe according to any one of claims 10 to 13, wherein the vibrating plate (14) applies a static force of from about 3.1 to 10.7 kN.

15. The process for finishing an impinged concrete coating on a pipe according to any one of claims 10 to 14, wherein the process is carried out at a surface speed of the pipe from about 50 to about 100 meters/min.

16. The process for finishing an impinged concrete coating on a pipe according to any one of claims 10 to 15, further comprising applying water on the concrete surface coating the pipe, preferably wherein water is applied prior to the scrapping step, and more preferably, wherein water is applied prior to the vibrationally compacting step.

17. The process for finishing an impinged concrete coating on a pipe according to claim 16, wherein the rate of water application is from 0.030 to 1.000 L/m².

## Patentansprüche

1. Rohrbeschichtungsendbearbeitungsvorrichtung (1), die Folgendes umfasst:
- einen oder mehrere Rahmen (2) mit einem ersten Arm (4) und einem zweiten Arm (6);
- ein Abziehelement (8), das mit einem ersten Arm (4) verbunden ist, um mit einem Rohr (12) in Eingriff zu gelangen, um in Bezug auf einen maximalen Rohrdurchmesser überschüssiges Material zu entfernen; und
- eine Vibrationsplatte (14), die mit einem zweiten Arm (6) verbunden ist, um eine aufgebrachte Betonbeschichtung (32) auf dem Rohr (12) zusammenzupressen,
wobei die Vibrationsplatte (14) erhöhte Ränder (20) umfasst, um zu verhindern, dass sich die Ränder der Vibrationsplatte (14) in die aufgebrachte Betonbeschichtung drücken.

2. Rohrbeschichtungsendbearbeitungsvorrichtung (1) nach Anspruch 1, die ferner eine Vibrationsvorrichtung (18) umfasst, die mit der Vibrationsplatte (14) verbunden ist.

3. Rohrbeschichtungsendbearbeitungsvorrichtung (1) nach Anspruch 1 oder 2, wobei die Vibrationsplatte (14) eine konkave Oberfläche (22) aufweist, die einen Krümmungsradius aufweist, um zu ermöglichen, dass die gesamte konkave Oberfläche (22) der Vibrationsplatte (14) in Kontakt mit einer Außenoberfläche des mit aufgebrachtem Beton beschichteten Rohrs (12) steht.

4. Rohrbeschichtungsendbearbeitungsvorrichtung (1) nach einem der Ansprüche 1 bis 3, wobei die Vibrationsplatte (14) und das Abziehelement (8) fluchtend entlang einer Achse im rechten Winkel auf die Längsachse des Rohrs (12) angeordnet sind.

5. Rohrbeschichtungsendbearbeitungsvorrichtung (1) nach einem der Ansprüche 1 bis 4, wobei das Abziehelement (8) eine erste Endplatte (24), eine zweite Endplatte (26) und eine Vielzahl von Stäben (28), die die erste Endplatte (24) und die zweite Endplatte (26) verbinden, aufweist; wobei die Vielzahl von Stäben (24) eine gekrümmte Ebene definieren, die einen Krümmungsradius aufweist, der einem festgelegten Maximalradius des beschichteten Rohrs (12) entspricht.

6. Rohrbeschichtungsendbearbeitungsvorrichtung (1) nach einem der Ansprüche 1 bis 5, die ferner Aufbringwalzen umfasst, die benachbart in Bezug auf die Vibrationsplatte (14) und das Abziehelement (8) angeordnet sind.

7. Rohrbeschichtungsendbearbeitungsvorrichtung (1) nach einem der Ansprüche 1 bis 6, wobei das Abziehelement (8) unterhalb und die Vibrationsplatte (14) oberhalb einer Ebene angeordnet ist, die das Rohr (12) diametrisch schneidet.

8. Rohrbeschichtungsendbearbeitungsvorrichtung nach Anspruch 7, wobei das Abziehelement (8) und die Vibrationsplatte (14) symmetrisch um die Ebene angeordnet sind, die das Rohr (12) diametrisch schneidet.

9. Rohrbeschichtungsendbearbeitungsvorrichtung (1) nach Anspruch 7 oder 8, wobei das Abziehelement (8) und die Vibrationsplatte (14) in einem Winkel von etwa 30° gemessen vom Mittelpunkt des Rohrs (12) angeordnet sind.

10. Verfahren zur Endbearbeitung einer aufgebrachten Betonbeschichtung auf einem Rohr (12) mit einer Vorrichtung (1) nach einem der Ansprüche 1 bis 9, wobei das Verfahren folgende Schritte umfasst:
- das Abziehen von Material, das in Bezug auf einen Maximaldurchmesser des beschichteten Rohrs überschüssig ist, und
- das Zusammenpressen einer Oberfläche des mit aufgebrachtem Beton beschichteten Rohrs (32) mittels Vibrationen zur Ausbildung eines geglätteten mit Beton beschichteten Rohrs (12).

11. Verfahren zur Endbearbeitung einer aufgebrachten Betonbeschichtung auf einem Rohr nach Anspruch 10, das ferner folgenden Schritt umfasst:
- das Aufbringen einer Betonbeschichtung auf eine Oberfläche eines Rohrs vor den Schritten des Abziehens und des Zusammenpressens mittels Vibrationen zum Erhalt des mit aufgebrachtem Beton beschichteten Rohrs (32).

12. Verfahren zur Endbearbeitung einer aufgebrachten Betonbeschichtung auf einem Rohr nach Anspruch 10 oder 11, wobei die Vibrationsplatte (14) einen Druck von etwa 34,47 bis etwa 5516 kPa (etwa 5 bis etwa 800 psi) aufbringt, wobei die Vibrationsplatte vorzugsweise mit einer Frequenz von etwa 1.500 bis etwa 18.000 Vibrationen/min vibriert.

13. Verfahren zur Endbearbeitung einer aufgebrachten Betonbeschichtung auf einem Rohr nach einem der Ansprüche 10 bis 12, wobei die Vibrationsplatte (14) eine Breite aufweist, die das zumindest zweimalige Zusammenpressen einer Oberfläche des mit aufgebrachtem Beton beschichteten Rohrs (32) ermöglicht.

14. Verfahren zur Endbearbeitung einer aufgebrachten Betonbeschichtung auf einem Rohr nach einem der Ansprüche 10 bis 13, wobei die Vibrationsplatte (14) eine statische Kraft von etwa 3,1 bis 10,7 kN aufbringt.

15. Verfahren zur Endbearbeitung einer aufgebrachten Betonbeschichtung auf einem Rohr nach einem der Ansprüche 10 bis 14, wobei das Verfahren mit einer Oberflächengeschwindigkeit des Rohrs von etwa 50 bis etwa 100 m/min durchgeführt wird.

16. Verfahren zur Endbearbeitung einer aufgebrachten Betonbeschichtung auf einem Rohr nach einem der Ansprüche 10 bis 15, das ferner das Aufbringen von Wasser auf die das Rohr beschichtende Betonoberfläche umfasst, wobei das Wasser vorzugsweise vor dem Schritt des Abziehens aufgebracht wird und wobei das Wasser noch bevorzugter vor dem Schritt des Zusammenpressens durch Vibrationen aufgebracht wird.

17. Verfahren zur Endbearbeitung einer aufgebrachten Betonbeschichtung auf einem Rohr nach Anspruch 16, wobei die Rate des Wasseraufbringens 0,030 bis 1,000 l/m² beträgt.

## Revendications

1. Dispositif de finition de revêtement de tuyau (1) comprenant :
- un ou plusieurs bâtis (2) ayant un premier bras (4) et un second bras (6) ;
- un racleur (8) couplé à un premier bras 4) destiné à venir en prise avec un tuyau (12) afin d'éliminer du matériau en excès d'un diamètre de tuyau maximum ; et
- une plaque vibrante (14) couplée à un second bras (6) pour compacter un revêtement de béton projeté (32) sur le tuyau (12),
dans lequel la plaque vibrante (14) comprend des bords en relief (20) afin d'empêcher les bords de la plaque vibrante (14) de s'enfoncer dans le revêtement de béton projeté.

2. Dispositif de finition de revêtement de tuyau (1) selon la revendication 1, comprenant en outre un vibrateur (18) couplé à la plaque vibrante (14).

3. Dispositif de finition de revêtement de tuyau (1) selon la revendication 1 ou 2, dans lequel la plaque vibrante (14) présente une surface concave (22) ayant un rayon de courbure pour permettre à toute la surface concave (22) de la plaque vibrante (14) de venir en contact avec une surface extérieure du tuyau revêtu de béton projeté (12).

4. Dispositif de finition de revêtement de tuyau (1) selon l'une quelconque des revendications 1 à 3, dans lequel la plaque vibrante (14) et le racleur (8) sont positionnés en ligne le long d'un axe perpendiculaire à l'axe longitudinal du tuyau (12).

5. Dispositif de finition de revêtement de tuyau (1) selon l'une quelconque des revendications 1 à 4, dans lequel le racleur (8) comporte une première plaque d'extrémité (24), une seconde plaque d'extrémité (26) et une pluralité de tiges (28) reliant la première plaque d'extrémité (24) à la seconde plaque d'extrémité (26) ; et la pluralité de tiges (24) définissant un plan incurvé ayant un rayon de courbure égal à un rayon maximum défini du tuyau revêtu (12).

6. Dispositif de finition de revêtement de tuyau (1) selon l'une quelconque des revendications 1 à 5, comprenant en outre des rouleaux de projection placés de manière adjacente à la plaque vibrante (14) et au racleur (8).

7. Dispositif de finition de revêtement de tuyau (1) selon l'une quelconque des revendications 1 à 6, dans lequel le racleur (8) est positionné en dessous et la plaque vibrante (14) est positionnée au-dessus d'un plan recoupant diamétralement le tuyau (12).

8. Dispositif de finition de revêtement de tuyau (1) selon la revendication 7, dans lequel le racleur (8) et la plaque vibrante (14) sont positionnés de manière symétrique autour du plan disséquant diamétralement le tuyau (12).

9. Dispositif de finition de revêtement de tuyau (1) selon la revendication 7 ou 8, dans lequel le racleur (8) et la plaque vibrante (14) sont positionnés selon un angle d'environ 30° mesuré à partir du centre du tuyau (12).

10. Procédé de finition d'un revêtement de béton projeté sur un tuyau (12) avec un dispositif (1) tel que défini dans l'une quelconque des revendications 1 à 9, le procédé comprenant les étapes consistant à :
- racler du matériau en excès d'un diamètre de tuyau revêtu maximum ; et
- compacter par vibrations une surface du tuyau revêtu de béton projeté (32) pour former un tuyau revêtu de béton lissé (12).

11. Procédé de finition d'un revêtement de béton projeté sur un tuyau selon la revendication 10, comprenant en outre l'étape consistant à :
- projeter un revêtement de béton sur la surface d'un tuyau, avant les étapes de raclage et de compactage par vibrations, pour obtenir le tuyau revêtu de béton (32).

12. Procédé de finition d'un revêtement de béton projeté sur un tuyau selon la revendication 10 ou 11, dans lequel la plaque vibrante (14) applique une pression d'environ 34,47 à environ 5516 kPa (environ 5 à environ 800 psi),
dans lequel la plaque vibrante vibre de préférence à une fréquence d'environ 1 500 à environ 18 000 vpm.

13. Procédé de finition d'un revêtement de béton projeté sur un tuyau selon l'une quelconque des revendications 10 à 12, dans lequel la plaque vibrante (14) a une largeur permettant de compacter, au moins deux fois, une surface du tuyau revêtu de béton projeté (32).

14. Procédé de finition d'un revêtement de béton projeté sur un tuyau selon l'une quelconque des revendications 10 à 13, dans lequel la plaque vibrante (14) applique une force statique d'environ 3,1 à 10,7 kN.

15. Procédé de finition d'un revêtement de béton projeté sur un tuyau selon l'une quelconque des revendications 10 à 14, dans lequel le procédé est mis en œuvre à une vitesse de surface du tuyau d'environ 50 à environ 100 mètres/minute.

16. Procédé de finition d'un revêtement de béton projeté sur un tuyau selon l'une quelconque des revendications 10 à 15, comprenant en outre l'application d'eau sur la surface de béton recouvrant le tuyau, de préférence dans lequel de l'eau est appliquée avant l'étape de raclage, et de manière plus préférée dans lequel de l'eau est appliquée avant l'étape de compactage par vibrations.

17. Procédé de finition d'un revêtement de béton projeté sur un tuyau selon la revendication 16,
dans lequel le débit d'application d'eau est de 0,030 à 1,000 L/m².
